

May 6, 1947.

G. T. RAYFIELD

2,420,014

CATHODE

Filed April 18, 1944



Fig. 3

*Improved Cathode*

Fig. 2

Fig. 1

INVENTOR.  
George T. Rayfield

BY *Harold E. Sorg*

ATTORNEY

## UNITED STATES PATENT OFFICE

2,420,014

## CATHODE

George T. Rayfield, San Bruno, Calif., assignor to  
Eitel-McCullough, Inc., San Bruno, Calif., a  
corporation of California

Application April 18, 1944, Serial No. 531,631

4 Claims. (Cl. 250—27.5)

## 1

My invention relates to a cathode for vacuum tubes.

It is among the objects of my invention to provide a cathode having improved electron emissive characteristics and superior physical properties.

The invention possesses other objects and features of advantage, some of which, with the foregoing, will be set forth in the following description of my invention. It is to be understood that I do not limit myself to this disclosure of species 10 of my invention, as I may adopt variant embodiments thereof within the scope of the claims.

Referring to the drawing:

Figure 1 is a vertical sectional view showing an electron tube having a filamentary cathode embodying my improvements; and

Figure 2 is an enlarged cross-sectional view of the improved filament wire.

Figure 3 is an enlarged sectional view of an indirectly heated cathode.

In terms of broad inclusion, my cathode comprises a core of material having good electron emissive properties, such as thorium, clad with a refractory metal, such as tantalum; the refractory metal sheath being preferably carburized. The method comprises first forming the cathode of the improved material, and then carburizing it. The cathode is mounted in an envelope with other suitable electrodes, the envelope being evacuated in any suitable manner.

In greater detail, and referring to the drawing, my cathode 2 is illustrated as filamentary type comprising a helical wire welded top and bottom to a pair of leads 3 sealed to stem 4 of envelope 6. It is understood however that the cathode may be of any suitable shape or structure, either directly or indirectly heated, as will be apparent to those skilled in the art.

Other components of the tube chosen for purposes of illustration include a tubular anode or plate 7 and a cage-type grid 8. The plate is supported on a lead 9 sealed to the upper end of the envelope by a bracket 11 secured to plate cap 12. Grid 8 is supported on rod 13 sealed to stem 4 by brackets 14, one of these rods serving as a lead. A base 16 cemented to the bottom of the envelope carries prongs 17 connected to cathode leads 3 by conductors 18 and to grid lead 13 by a conductor 19.

While I have shown my cathode in a triode combination, it is understood that it may be embodied in other tube types such as a diode or multi-grid tubes.

Now going to the cathode or thermionic emitter element from which electrons are evaporated. As

shown in Figure 2, the filament wire comprises a composite strand having a core 21 clad with a sheath 22. Core 21 is of a material having good electron emissivity, which would include generally those materials having a low work function such as thorium, uranium and barium, thorium being preferred. In the filament illustrated the core is a solid rod composed essentially of metallic thorium, preferably having a diameter about half that of the overall wire diameter. This has the advantage of being able to draw the final composite wire in an ordinary wire machine.

If desired however the core may be of powdered metallic thorium compressed into the tubular outer sheath. Also, the core may be a composition or alloy of metallic thorium with another metal, or a compound such as thorium carbide. In any case however the core is a distinct homogeneous body forming the central zone of the wire, and provides within the filament wire an ample reservoir of the highly emissive or active material.

Sheath 22 is of a refractory metal such as tantalum or molybdenum. Tantalum is preferred for several reasons, one being that it is ductile enough to be readily drawn as a sheath over the core in a wire machine. Tantalum also provides a good medium through which the thorium is able to migrate to the surface of the wire, from which surface the electrons are emitted.

Sheath 22 is also preferably carburized. This is accomplished by heating the cathode in an atmosphere containing a hydrocarbon, similar to the process of carburizing an ordinary tungsten filament, whereby carbon is taken up by the sheath in the form of tantalum carbide. This carburization further improves the emissive properties of the cathode.

My improved cathode is superior to the usual thoriated tungsten filament wherein finely divided thoria (thorium oxide) is distributed throughout a tungsten wire. In making this ordinary thoriated tungsten wire it is difficult to control the distribution of the thoria, resulting in a bad manufacturing problem and nonuniformity in the final product. This is overcome in my cathode element. Furthermore my improved emitter element provides a reservoir of the active agent, insuring longer life of the filament. Still further, my improved filament has greater mechanical strength and is less brittle than an ordinary thoriated tungsten filament. This is very important because many tubes are lost during manufacture and subsequent operation because of filament breakage.

My improved emitter element is also adaptable

for use in an indirectly heated type of cathode. As shown in Figure 3, the element is formed as a sheet with a core layer 26 of metallic thorium interposed between sheath layers 27 of a refractory metal. Tantalum is particularly preferred as the sheath in this case because of its ductility in rolling and otherwise fabricating the composite sheet. The sheet may then be shaped as a tube or cylinder for encircling a heater 28.

My improved cathode is not to be confused with composite elements in the past wherein a layer of material containing barium or strontium oxide is formed on the surface, or where the inner portion of the element is of a refractory metal having thorium oxide distributed in it.

I claim:

1. A cathode for electron tubes comprising a thorium core clad with tantalum.
2. An indirectly heated cathode comprising a tubular emitter element of sheet material having a core layer of thorium interposed between sheath layers of tantalum.
3. A sheet material for cathodes comprising a core layer composed essentially of metallic thorium interposed between sheath layers of a refractory metal.

4. An indirectly heated cathode for electron tubes comprising a tubular emitting element consisting essentially of tantalum and thorium, and a heater disposed within said element.

GEORGE T. RAYFIELD.

#### REFERENCES CITED

The following references are of record in the file of this patent:

#### UNITED STATES PATENTS

| Number       | Name           | Date          |
|--------------|----------------|---------------|
| 1,663,547    | Gero           | Mar. 27, 1928 |
| 1,695,819    | O'Neill        | Dec. 18, 1928 |
| 15 1,961,122 | Lowry          | May 29, 1934  |
| 1,917,991    | McCullough     | July 11, 1933 |
| 1,894,059    | Ruffley        | Jan. 10, 1933 |
| 2,091,554    | Mendenhall     | Aug. 31, 1937 |
| 1,948,445    | Lederer        | Feb. 20, 1934 |
| 1,957,486    | Becker         | May 8, 1934   |
| 2,140,534    | Mahoney        | Dec. 20, 1938 |
| 2,107,945    | Hull et al.    | Feb. 8, 1938  |
| 2,175,345    | Gaidies et al. | Oct. 10, 1939 |